

## UNITED STATES PATENT OFFICE

ROBERT PETITDIDIER AND FRANÇOIS VICTOR FEYNIER, OF PARIS, FRANCE, ASSIGNEES  
TO ETABLISSEMENTS PETITDIDIER (ANCIENNE MAISON JOLLY-BELIN), OF ST.-  
DENIS, FRANCE

## COLOR PRINTING PROCESS FOR TEXTILE FABRICS

No Drawing. Application filed July 12, 1926, Serial No. 122,039, and in France August 1, 1925.

The present invention has for its object a color printing process for textile fabrics of a composite character, which essentially consist on the one hand of artificial silk made of 5 acetate of cellulose, and on the other hand of cotton, flax, natural silk, wool, or artificial fibres such as viscose silk, and the fabric may comprise the whole or a part of these various fibres.

10 The said process is based upon a most striking observation that certain colors having anthraquinone as a base, such as the amino hydroxy, diamino, tetramino, methyl-amino and di-methyl-diamino colors, certain 15 of which are known in commerce under the names of 1 amino 2 methyl anthraquinone, 1 methyl amino anthraquinone, 1 amino 4 hydroxy anthraquinone, 1.4 diamino anthraquinone, 1.4.5.8.tetra amino anthraquinone, 20 1.4 diamino dimethyl anthraquinone and dinitro diphenylamine, when printed upon composite fabrics, will react differently during the course of a fixing which is effected in determined conditions of duration and temperature, firstly upon the acetate of cellulose 25 fibres, and secondly upon the other fibres whether animal, vegetable or artificial, and that furthermore, the cellulose acetate silk is but little affected by the action of the reducing agent which consists of sodium hydrosulfite, whereas on the contrary, under the 30 action of the said reducing agent, the said colors will disappear almost entirely from all the other fibres, so that by printing upon 35 the said composite fabrics, we are enabled to obtain an appearance different from what is offered by the known methods. In particular, these fabrics show multi-colored or variegated effects upon similar cellulose acetate threads to the exclusion of the other threads of the fabric.

Certain of the acid colors such as citronine (diazoted sulfanilic acid + diphenylamin strongly nitrated) and rocceline (diazoted 45 naphthionic-acid + betanaphthol), soluble blue for silk (disulfonated triphenyl-para-ros aniline), and certain basic colors after a preliminary mordanting of the fabric with tannin or acetanol (pyridine nitrate), have the 50 same properties.

The color printing process comprises the following operations, in the case of fabrics consisting of a mixture of cellulose acetate silk and viscose silk or cotton forming the backing.

(a) We begin by printing on the fabric 55 any suitable pattern, in the known manner, employing the aforesaid colors.

(b) The printed fabric is treated in a steam operated autoclave for fixing the 60 colors. During this operation, the color becomes fixed upon the cellulose acetate fibre, but it is only incompletely fixed upon the cotton backing and upon the viscose silk.

(c) The fabric is then rinsed. During this 65 operation, a part of the colors, which impregnated the cotton backing and the viscose will be removed.

(d) The fabric is finally treated in a sodium hydrosulfite bath, containing 1 gram of hydrosulfite per liter of water, the bath being heated to about 75 degrees C. During this 70 operation, the color will be discharged from all parts of the fabric except the cellulose acetate fibres.

The fabric can be utilized in this condition, 75 or it may be treated in a dye bath which acts upon the cotton backing, without any marked change in the color of the cellulose acetate.

In a modification of our said process, we 80 dispense with the sodium hydrosulfite bath, i. e. the fabric is utilized in the state in which it appears at the end of operation (c), for in these conditions we already obtain an excellent effect of color upon color.

When the fabric to be printed has a backing of natural silk, we prefer to increase the amount of hydrosulfite from 1 to 2 or 3 grams per liter of water, according to the quality of the silk. In this manner the color of the 85 natural silk backing is diminished, whereas the colors printed on the cellulose acetate silk with dyestuffs having anthraquinone as a base as above specified will preserve their brilliancy, and will assume suitable shades according to the duration and the temperature of the treatment.

Another feature consists in the fact that we may efface the traces of color which still exist upon the backing, by treating the fabric 90 100

in a bath containing 0.001 by volume of sulfuric acid at 66 degrees Bé., the bath having preferably a temperature of 80 degrees C.

It may happen that by reason of the strength of the colors employed for printing the acetate of cellulose, the backing which should be white may still remain slightly colored, which may be prejudicial to the appearance of the fabric when the backing is not 5 to 10 to be covered by an additional dyeing. However by treating the fabric—after printing the cellulose acetate as above disclosed—in a bath of potassium permanganate and then in a solution of sodium bisulfite, the traces of 15 color which somewhat stain the backing will entirely disappear.

The proportions to be adopted, which are given by way of example, are 20 to 25 grams of potassium permanganate in a bath of 100 20 grams of water, and the density of the sodium bisulfite solution may be about 15 degrees Bé.

In the same manner as for the fabrics with a cotton backing, the fabric thus prepared may be treated in a dye bath which acts upon 25 the natural silk backing, without any marked change in the color imparted to the cellulose acetate. With fabrics having a wool backing, we prefer to increase the strength of the hydro sulfite bath to 5 grams per liter of water. 30 We thus obtain upon the wool backing a sufficient attenuation of the printing to obtain, by a subsequent dyeing, a uniform backing, and the shades of color upon the acetate of cellulose will always preserve their original 35 brilliancy.

Obviously, the aforesaid process is susceptible of various modifications in its execution, without departing from the spirit of the invention. In particular, the indications concerning the proportions and temperatures 40 may be modified.

What we claim is:

1. A color printing process for composite fabrics composed of cellulose acetate artificial silk mixed with other suitable fibers 45 which consists in printing the fabric with colors of an anthraquinone base adapted to produce dyeing reactions upon the cellulose acetate, fixing the printed colors and rinsing 50 the fabric in a reducing bath for removing all color from the fibers which are not the cellulose acetate fibers.

2. A color printing process for composite fabrics composed of cellulose acetate artificial silk mixed with other suitable fibers 55 which consists in printing the fabric with colors of an anthraquinone base adapted to produce dyeing reactions upon the cellulose acetate, fixing the printed colors and rinsing 60 the fabric in a bath of sodium hydrosulfite for removing all color from the fibers which are not the cellulose acetate fibers.

3. A color printing process for composite fabrics composed of cellulose acetate artificial silk mixed with other suitable fibers 65

which consists in printing the fabric with colors of an anthraquinone base and adapted to produce dyeing reactions upon the cellulose acetate, fixing the printed colors, rinsing the fabric in a reducing bath for removing all color from the fibers which are not the cellulose acetate fibers and subsequently dyeing the fabric in a bath which reacts upon the fibers of the fabric without changing the color of the cellulose acetate fibers. 70 75

4. A color printing process for composite fabric of cellulose acetate artificial silk mixed with other suitable fibers which consists in printing the fabric with colors of an anthraquinone base adapted to produce dyeing reactions upon the cellulose acetate, fixing the printed colors, rinsing the printed colors, rinsing the fabric in a bath of sodium hydrosulfite containing from 1 to 5 grams of hydrosulfite per liter of water for removing all the color from the fibers 80 85 which are not the cellulose acetate fibers.

5. A color printing process for composite fabrics composed of cellulose acetate artificial silk mixed with other suitable fibers, which comprises printing the fabric with 90 colors of an anthraquinone base adapted to produce dyeing reactions upon the cellulose acetate, fixing the printed colors and rinsing the fabric successively in a bath of sodium hydrosulfite, in a bath of potassium permanganate and in a solution of sodium bisulfite, for removing all color from the fibers which are not the cellulose acetate fibers. 95

6. A color printing process for composite fabrics composed of cellulose acetate artificial silk mixed with other suitable fibers, which comprises printing the fabric with colors of an anthraquinone base adapted to produce dyeing reactions upon the cellulose acetate, fixing the printed colors and rinsing the fabric successively in a bath of sodium hydrosulfite, in a bath of potassium permanganate containing from 20 to 25 grams of permanganate for 100 grams of water and in a sodium bisulfite solution having a density of about 15 degrees Bé. for removing all color from the fibers which are not the cellulose acetate fibers. 100 105 110 115

In testimony whereof we affix our signatures.

ROBERT PETITDIDIER.  
FRANÇOIS VICTOR FEYNIER.